

## 1

3,545,074  
METHOD OF MAKING COPPER  
ALLOY PRODUCTS

George S. Foerster and Garth D. Lawrence, Midland, Mich., assignors to The Dow Chemical Company, Midland, Mich., a corporation of Delaware  
No Drawing. Filed July 29, 1968, Ser. No. 748,176  
Int. Cl. B23p 17/00, 25/00

U.S. CL. 29—527.7

6 Claims

## ABSTRACT OF THE DISCLOSURE

A method of preparing copper alloy products which comprises dissolving solid insoluble elements or compounds in molten copper or copper alloy in an amount sufficient to provide upon solidification from about 1 to about 30 percent by volume of dispersed second phase; rapidly solidifying the resultant copper alloy, thereby forming pellets; and working the pellets to form a copper alloy product.

## BACKGROUND OF THE INVENTION

## Field of the invention

The invention relates to a method of preparing a high strength, wrought copper alloy product.

For the purposes of the specification and claims the term "copper" as used herein includes both copper metal and copper base alloys. Copper base alloys are understood to be alloys in which the copper content, by weight is greater than the content of any single component of the alloy. Preferably the alloy comprises at least about 70 weight percent of copper. For applications requiring good conductivity Cu content of at least 90% is preferred.

## Prior art

A major reason for using copper in a wide variety of applications is its good thermal and electrical conductivity which is at a maximum in the pure or unalloyed state. However, copper is relatively weak in this condition. Conventionally copper has been strengthened by the addition of solid solution hardeners such as one or more of the metals zinc, tin, silicon, and aluminum in various combinations and various proportions. Copper alloys have been further improved by the addition of elements such as beryllium or mixtures such as aluminum and iron whereby precipitation hardening takes place, normally during heat treating of the solidified metal. Such metals are sometimes called age hardeners when added to copper. However such alloy additions, or merely working the unalloyed copper, significantly reduces the conductivity. Furthermore, the strengthening afforded by these conventional techniques is rapidly lost at elevated temperatures.

Considerable attempts have been made to produce a dispersion hardened copper alloy, i.e., an alloy having stable, micron sized second phase particles. The conventional method of dispersion hardening is to simply mix the solid insoluble particles with copper powder, compact the mixture, and hot work the compact. However, in order to achieve the desired dispersion hardening effect, the second phase particles must be extremely small. Thus, heretofore dispersion hardening of copper and copper alloys has been very difficult and expensive.

A primary object of the present invention is to provide a method for strengthening copper at room and elevated temperatures without serious loss of conductivity characteristic of the conventional method. A further object of the present invention is to provide an improved method for dispersion hardening copper alloys.

## 2

## SUMMARY OF THE INVENTION

These and other objects and advantages are obtained in the method of the present invention which comprises: dissolving in molten copper a sufficient amount of dispersion hardening material to provide upon solidification from about 1 to about 30 percent by volume, ordinarily from about 2 to about 20 percent by volume, and preferably from about 4 to about 10 percent by volume, of solid insoluble second phase in the copper matrix; rapidly solidifying the resultant molten copper alloy, e.g., by atomizing, to form pellets; and working the pellets to produce a high strength wrought copper alloy product. Such product has relatively high room and high temperature strength properties, thermal conductivity and electrical conductivity.

Dispersion hardening is differentiated from precipitation hardening on the basis that the second phase formed on dispersion hardening (1) generally separates during solidification of the alloy, though it may separate from under cooled supersaturated solid solution as a consequence of working the alloy, (2) is comprised of particles having dimensions in the micron range rather than the Angstrom range, and (3) is substantially not solid soluble in the matrix metal during conventional heat treatment of the alloy; therefore agglomeration tends to be mineral.

The dispersion hardening material should have appreciable liquid solubility but limited solid solubility and/or diffusivity so that after hot working, exposure to high temperatures, or solution heat treatment of the dispersion hardened metal, the dispersion hardening material, once intimately dispersed in the solid metal, remains uniformly dispersed as particles less than about 5 microns in diameter, and preferably less than about 1 micron in diameter. The term diameter is intended to refer to the longest dimension of the particle in the event that the particle is not equiaxed. The most preferred dispersion hardening materials are compounds that are stable in the matrix or base metal, have very high melting temperatures, but have limited solid solubility.

The second phase should be stable, i.e., it should agglomerate relatively slowly if at all in the copper alloy. Materials that have high melting temperatures, above about 2500° F. and preferably above about 3000° F., tend to be stable. Another indicator of stability is solid solubility, which should be below about 2 atomic percent and more preferably below about 1 atomic percent. Also, the second phase should not significantly depress the solidus of the copper or copper alloy in order not to impair hot workability or maximum service temperature.

For purposes of the specification and claims, compounds formed by a metal and metalloid are herein referred to as intermetallic compounds. Such compounds may be added per se to the molten copper or formed in situ. Chemical compounds such as Cu<sub>2</sub>O may also be formed in situ. The dispersion hardening material, whether it is functioning as an elemental substance, intermetallic compound, or other compound, should have sufficient liquid solubility to permit incorporation of useful proportions in the molten copper. Therefore, liquid solubility should be at least 1 atomic percent and preferably at least 3 atomic percent.

Broadly speaking, the addition to the copper source, i.e., copper or copper alloy, of dispersion hardening material in the form of one or more chemical elements or compounds in an amount that is miscible with the molten alloy but forms a second phase on solidification of the alloy or as a consequence of subsequent working, brings about the desired strengthening of the copper alloy and thorough dispersion of the second phase according to the invention. The solid solubility of the second phase may

be exceeded because the addition solubility per se has been exceeded, or on account of interaction between different elements constituting the addition, or between the addition and the copper of the alloy, to form one or more compounds present in an amount in excess of solubility thereof.

Suitable elements for addition to form copper compounds of limited solid solubility include for example cerium and other rare earth metals and mixtures, thorium, zirconium, boron, calcium, and sulfur. Such elements have a solid solubility in copper below about 2 atomic percent.

Elements that react in copper to form a phase having limited solid solubility are tabulated in the following Groups I and II. Each of the elements in Group I react with most of the elements in Group II to form the desired phase and vice versa.

## Group I:

Titanium  
Zirconium  
Rare earth metals  
Scandium  
Yttrium  
Calcium

## Group II:

Boron  
Silicon  
Phosphorous  
Arsenic  
Antimony

Examples of stable intermetallic compounds suitable for dispersion hardening according to the method of the present invention and formed of the consequences of such interactions are:  $\text{Ca}_3\text{As}_2$ ,  $\text{Ti}_5\text{Si}_3$ ,  $\text{CeSb}$ , and  $\text{ZrB}_2$ .

Preferred additions that bring about dispersion hardening in the copper or copper base alloy included, for example, thorium, rare earth metal mixtures,  $\text{ZrB}_2$  and  $\text{Ti}_5\text{Si}_3$ .

In dissolving the dispersion hardening elements in the molten copper, conventional alloy and melting techniques as practiced by those skilled in the art, may be employed. The alloying constituents may contain those amounts and types of impurities normally found therein.

To obtain the benefits of the solid insoluble second phase material it is essential that the second phase material be finely and intimately dispersed throughout the solidified copper metal. Rapid solidification, such as by atomizing, is a key step in the preparation of the copper alloy product. The homogeneous melt of copper containing dispersion hardening material, with or without solution hardening metals and precipitation hardening metals, is rapidly solidified, e.g., by atomizing the molten metal as fine droplets in gas so that droplets solidify therein. If desired, the droplets may be projected against a relatively cold metal surface, preferably contacting a cold metal surface before the liquidus temperature has been reached in the droplet, in order to provide more rapid cooling and even finer distribution of the second phase material. In some cases, the alloy may super cool and solidify without separation of the second phase. In that event, the second phase will generally form and separate during or subsequent to wrought operation in which the atomized particles are employed.

On carrying out rapid solidification by atomizing into a gas environment, it is desirable to utilize pellets small enough to pass through a 100 mesh sieve (U.S. Standard Sieve series) although pellets as coarse as about 20 mesh are satisfactory. Use of such fine pellets assures sufficient dispersion of the second phase material during solidification of the pellet. The pellets may be collected in water below the gaseous environment but this is gener-

ally to be avoided since some surface oxidation of the pellets may occur. Such oxidation tends to interfere with bonding of the pellets during subsequent compacting and working.

The pellets can then be worked by extrusion, forging, or other conventional pellet fabricating techniques at room or elevated temperatures to form a copper alloy product characterized by a fine second phase dispersion in the copper matrix, i.e., a dispersion hardened copper base alloy. Preferably the pellets are worked by extrusion.

The present invention provides a method of preparing a dispersion hardened copper alloy having the desired characteristics of both room temperature and high temperature strength with adequate conductivity. This copper alloy product is obtained without employing the extremely fine powders conventionally used with their attendant difficulties.

The following examples serve to illustrate the invention and are not intended to limit the scope thereof.

## EXAMPLE 1

A melt of a copper alloy containing 0.53 weight percent misch metal (Example 1) was prepared and jet atomized using an argon atmosphere to form pellets passing through a 100 mesh screen. The pellets were cold compacted

in a 3 inch extrusion press container and heated to 1000° F. However, the compact could not be extruded into  $\frac{1}{2}$  inch diameter rods using 500 tons extrusion pressure. The hot pressed billet was ejected, cooled and machined to fit into a  $\frac{2}{3}$  inch O.D. x  $2\frac{1}{2}$  I.D. copper tube. The canned alloy was then heated to 1500° F. and extruded at 30 feet per minute into  $\frac{1}{2}$  inch diameter rods from an extrusion container maintained at 1000° F. After removal from the copper tube the extruded rod, a copper alloy product made by the method of the present invention, had the following tested room temperature properties: 37 percent elongation (%E), 20K s.i. tensile yield strength (TYS), and 36K s.i. tensile strength (TS).

For comparison a copper alloy containing 2.44 weight percent misch metal (comparative example) was conventionally cast into 3 inch diameter billets. The billets were extruded at 30 feet per minute into  $\frac{1}{2}$  inch diameter rods; one at 1000° F., one at 1500° F. The rod extruded at 1500° F. had the following tested room temperature properties: 32% E, 13K s.i. TYS and 41K s.i. TS.

The copper alloy pellet extrusion product of the present invention was compared metallographically with the conventional ingot extrusion (both extruded at 1500° F.). The pellet extrusion was only partially recrystallized while the ingot extrusion was completely recrystallized. This difference is also reflected in the higher TYS of the pellet extrusion product. Annealing the pellet extrusion for one hour at temperatures up to 1500° F. had no effect on the structure. Even after annealing at 1900° F. the recrystallization of the pellet extrusion was incomplete. Grain size of the pellet extrusion remained relatively fine (about 1 mil or less) in spite of annealing.

The data presented show that the method of the present invention produces a fine dispersion of solid insoluble second phase, i.e., dispersion hardening, which inhibits recrystallization and grain growth, and has high resistance to deformation at elevated temperature, e.g., 1000° F.

Further, the pellet extrusion (Example 1) and the comparative example were measured for creep resistance at elevated temperatures. Table I shows the results of such creep tests.

TABLE I

| Example No.      | Temp.,<br>°F. | Time,<br>hrs. | Percent creep at— |           |            |          |
|------------------|---------------|---------------|-------------------|-----------|------------|----------|
|                  |               |               | 5K s.i.           | 7.5K s.i. | 11.5K s.i. | 15K s.i. |
| Comparative----- | 600           | 100           | 0.036             | 0.11      | 0.86       | -----    |
|                  | 600           | 1,000         | 0.082             | 0.38      | 3.26       | -----    |
|                  | 800           | 100           | 1.72              | -----     | -----      | -----    |
|                  | 800           | 1,000         | 12.6              | -----     | -----      | -----    |
| 1-----           | 600           | 100           | 0.021             | 0.025     | 0.14       | 0.53     |
|                  | 600           | 1,000         | 0.024             | 0.028     | 0.16       | 1.19     |
|                  | 800           | 100           | <0.01             | <0.01     | -----      | -----    |
|                  | 800           | 1,000         | 0.02              | 0.06      | -----      | -----    |

The alloy made of the present invention shows substantially improved high temperature creep properties over the conventional alloy. For instance the comparative example had 3.26% creep after 1000 hours at 600° F. while Example 1 had only 0.16% creep.

## EXAMPLES 2-5

Various copper alloys containing solid insoluble second phase were melted and atomized into discrete particles by splattering the droplets onto a cold, metallic surface. The resultant particles were extruded from a  $\frac{3}{4}$  inch diameter container into a  $\frac{1}{4}$  inch diameter rod at about 1450° F. The rods made by the method of the present invention were tested at room and elevated temperatures. Table II reports various properties of these alloys including %E, TS, yield strength (YS), and electrical conductivity.

For comparison purposes a copper base alloy was prepared and cast into a 3 inch diameter billet which was then extruded into a  $\frac{1}{4}$  inch diameter rod at 1450° F.

TABLE II

| Example No.       | Nominal composition <sup>1</sup> | YS at 70° F. | At 1,000° F. |    |    | Electrical conductivity, $10^3$ mhos./cm. <sup>3</sup> | Copper conductivity equivalent, percent <sup>4</sup> |
|-------------------|----------------------------------|--------------|--------------|----|----|--------------------------------------------------------|------------------------------------------------------|
|                   |                                  |              | %E           | YS | TS |                                                        |                                                      |
| Comparative ingot | 2.3 Ti, 0.5B                     | 28           | 34           | 5  | 8  | 4.60                                                   | 78.5                                                 |
| 2.                | 3 Zr                             | 28           | 33           | 14 | 19 |                                                        |                                                      |
| 3.                | 3 Th                             | 41           | 5            | 10 | 12 |                                                        |                                                      |
| 4.                | 3 MM <sup>2</sup>                | 35           | 4            | 14 | 17 | 5.24                                                   | 89.5                                                 |
| 5.                | 2.3 Ti, 0.5B <sup>3</sup>        | 32           | 33           | 20 | 26 |                                                        |                                                      |

<sup>1</sup> Weight percent; balance being essentially copper.

<sup>2</sup> Misch metal 35 to 80 weight percent Ce, up to 5 percent non-rare earth metal, balance being other rare earth elements.

<sup>3</sup> Heat treated 1 hour at 1,000° F. before testing.

<sup>4</sup> Conductivity of elemental copper is  $5.85 (10^3)$  mhos./cm.<sup>3</sup>.

The data of the table demonstrates that the method of the present invention produces a copper alloy product which has substantial room temperature and high temperature strength without a significant loss in conductivity. For example, Example 5 has a yield strength of 4 times that of the comparative alloy although the compositions are the same.

In a like manner other dispersion hardeners as that term has been explained and defined in the specification may be dissolved in molten copper and copper alloys including precipitation hardened alloys, the alloy melt rapidly solidified to form pellets, and the resulting pellets worked to form a copper alloy product which has high strength at room and elevated temperatures plus sufficient conductivity.

The method of the present invention having thus been fully described, various modifications thereof will be at once apparent to those skilled in the art. The scope of the invention is to be considered limited only by the breadth of the claims herein appended.

We claim:

1. A method of preparing a high strength, wrought copper alloy product which comprises:

(a) dissolving in molten copper an amount of at least

one dispersion hardening material sufficient to provide upon solidification from about 1 to about 30 volume percent of second phase;

(b) rapidly solidifying the resultant molten copper alloy into pellets containing said dispersion hardening material as a second phase; and

(c) working the pellets to form a high strength, wrought copper alloy product; such product being further characterized as containing the second phase dispersed therethrough as particles not exceeding 5 microns in maximum dimension.

2. The method of claim 1 employing at least two dispersion hardening materials wherein at least one of said dispersion hardening materials is selected from the group consisting of calcium, titanium, zirconium, thorium and rare earth mixtures; and at least one of said dispersion hardening materials is selected from the group consisting of boron, silicon, phosphorous, arsenic and antimony.

3. The method of claim 1 wherein the amount of dispersed second phase is from about 2 to about 20 volume

percent and the second phase particle size in the wrought copper alloy product is less than about 1 micron in maximum dimension.

4. The method of claim 1 and including the step of atomizing the molten resultant copper alloy into droplets thereof to provide rapid solidification into said pellets.

5. The method of claim 4 and including the step of projecting the atomized droplets against a cold, conductive surface thereby to solidify said droplets.

6. The method of claim 1 wherein the working of the solidified resultant alloy pellets is carried out by extrusion.

## References Cited

## UNITED STATES PATENTS

50 3,138,851 6/1964 Radtke et al. ----- 29—182  
3,286,334 11/1966 Hay ----- 29—527.7

JOHN F. CAMPBELL, Primary Examiner

55 D. C. REILEY, Assistant Examiner

U.S. Cl. X.R.

29—420.5; 164—76